

Patented May 21, 1940

2,201,488

## UNITED STATES PATENT OFFICE

2,201,488

## PROCESS OF PICKLING METALS

Marion W. Harman, Nitro, W. Va., assignor to  
Monsanto Chemical Company, St. Louis, Mo.,  
a corporation of Delaware

No Drawing. Application October 5, 1938,  
Serial No. 233,477

16 Claims. (Cl. 148-8)

The present invention relates to the cleaning of metallic surfaces and particularly to a new class of steel pickling inhibitors which are employed to prevent undue attack upon the surface 5 of a metal when in contact with a pickling bath of an acid nature.

Pickling solutions for removing oxides from the surface of metals ordinarily consist largely of a dilute solution of an inorganic acid such as 10 sulfuric or hydrochloric acid. The acid although it dissolves the oxides and scale, also attacks the metal to some extent so that the acid is largely consumed and a certain amount of metal is lost. It also appears that the hydrogen liberated by 15 the action of the acid on the metal has a serious embrittling effect upon the metal being treated. The escaping hydrogen also carries with it a fine spray of the acid liquor from the pickling bath which produces an atmosphere possessing corrosive properties and one which is injurious to 20 health and damaging to equipment.

By the present invention, these objectionable features of the pickling process are substantially overcome or reduced to a minimum. More 25 specifically, some of the objects of the present invention are to obviate over-pickling, embrittlement and pitting of the articles treated; to minimize the amount of metal lost in pickling; to increase the efficiency of the pickling operation; 30 to prolong the effective life of the pickling bath; and particularly to facilitate the pickling operation. Other and further objects of the invention will be apparent from the following description and accompanying examples.

To accomplish to as great an extent as possible 35 the objects set forth in accordance with the present invention, there is added to the pickling bath an inhibitor or regulating agent which acts to restrain the action of the acid from attacking clean metal but assists in removing the rust, scale, and other deposits or in other words the inhibitor causes the acid selectively to remove such materials without appreciably attacking the clean portions of the metal under treatment.

The new class of pickle regulators comprise 45 the esters of thiocarbamic acids and are commonly referred to as thiourethanes. Except for the N-alkyl compounds which are liquids, they are usually solid crystalline compounds of relatively low melting point. One method for their preparation is by the action of ammonia or an 50 amine on a xanthic ester although other methods have been described in the chemical literature and may be employed when desired. One precaution to be observed, whatever the method of preparation, is that the thiourethanes, while relatively stable compounds in other respects, readily undergo oxidation in the presence of mild oxidizing agents and should not be heated in the

presence of oxidizing mineral acids nor in the presence of excess caustic soda which catalyzes their decomposition. The thiourethanes are a well known class of compounds and the present invention in nowise relates to their preparation 5 nor is it limited thereto.

In order to further illustrate the class of compounds to which the present invention pertains, the thiourethanes are designated by the following structural formula



wherein R<sub>1</sub> and R<sub>2</sub> represent hydrogen, alkyl, 15 aralkyl and carbocyclic groups, the latter term including typical aryl groups and hydrogenated aryl groups and R<sub>3</sub> represents an ester forming radical such as alkyl, aralkyl and carbocyclic groups, the latter term likewise including typical 20 aryl and hydrogenated aryl groups.

Typical examples of the preferred class of compounds are



As specific embodiments of the invention which are to be understood as illustrative of the invention and not limitative thereof, typical examples of the preferred class of materials were employed 5 in the metal pickling process under conditions which duplicated, so far as possible those commonly followed in commercial practice. A portion of one of the preferred class of compounds was incorporated in a pickling bath and its value 10 as an inhibitor determined in the following manner: A test piece of 28 gauge hot rolled tin plate steel stock, approximately 4" x 3" in dimension, was immersed in the pickling bath comprising substantially 750 c. c. of a water solution 15 containing approximately 6% by weight of 66° Bé. sulfuric acid and a small amount of one of the inhibitors above described. The temperature of the bath was maintained at substantially 82° C. The steel test piece after thoroughly 20 cleaning was weighed before immersion in the bath, and after 40 minutes pickling the test piece was again weighed, the difference between the two weights representing the metal loss during 25 pickling. The metal loss per square inch of surface exposed compared with the metal loss per square inch of surface exposed of a similar test piece treated in an analogous manner but without the use of any inhibitor provides a measure 30 of the inhibiting value of the compound employed. The results obtained upon testing typical examples of the preferred class of materials are given in the following table. 0.234 gram of inhibitor was employed in testing thiourethane itself and in every other case 0.0936 gram of 35 inhibitor was employed.

Table I

| 40 | Inhibitor employed                         | Weight of metal before test in grams | Weight of metal after test in grams | Total loss of metal in grams | Metal loss per square inch of surface exposed |
|----|--------------------------------------------|--------------------------------------|-------------------------------------|------------------------------|-----------------------------------------------|
|    | N-phenyl thiourethane                      | 21.3808                              | 21.3414                             | 0.0394                       | .001641                                       |
| 45 | N-cyclohexyl thiourethane                  | 23.2207                              | 23.2114                             | 0.0093                       | .000387                                       |
|    | Thiourethane                               | 24.3387                              | 24.2330                             | 0.1057                       | .004404                                       |
|    | N-phenyl $\beta$ hydroxyethyl thiourethane | 22.9161                              | 22.8864                             | 0.0297                       | .001237                                       |
|    | N-phenyl benzyl thiourethane               | 23.3690                              | 23.3535                             | 0.0155                       | .000645                                       |
| 50 | N-p-diphenyl thiourethane                  | 22.5100                              | 22.4900                             | 0.0200                       | .000833                                       |
|    | N-phenyl butyl thiourethane                | 23.1478                              | 23.1368                             | 0.0110                       | .000458                                       |
|    | N- $\alpha$ -naphthyl thiourethane         | 23.5199                              | 23.5098                             | 0.0101                       | .000420                                       |
|    | Blank                                      | 22.2020                              | 21.6333                             | 0.5637                       | .0234                                         |

55 It is apparent from the data set forth that the preferred class of materials constitute an important and highly efficacious group of inhibitors as in all cases wherein one of the preferred inhibiting compounds was incorporated in the pickle liquor there resulted a great saving in the loss in weight of the steel test strips as compared with that resulting when no inhibitor was employed.

Other modes of employing inhibitors of the 65 class hereinbefore set forth in the acid pickling of metals are apparent to those skilled in the art to which the invention pertains. The products described may be employed in the presence of foaming agents, ionizable substances or other 70 materials ordinarily used. Thus the preferred class of materials may be employed as the sole inhibitor or they may be employed in conjunction with other materials exhibiting an inhibiting action or with inert fillers, dispersing agents, etc. For example the preferred class of mate-

rials were found to be particularly effective when employed in small quantities in conjunction with another known inhibitor and inert filling material whereby the preferred material although present as a minor proportion of the composition exhibited marked activating action so that the combined inhibiting action was superior to that of any ingredient alone. It is thus apparent that the preferred class of pickling inhibitors may be employed in a variety of useful ways and numerous modifications of the invention suggest themselves whereby improved results would be obtainable by employing the preferred thiourethanes either as the sole inhibitor, as an activator for other known inhibitors or in conjunction with non-inhibiting ingredients exhibiting other useful properties in the pickling bath. In addition the inhibitors of this invention are definite chemical compounds and are readily reproducible so that it is possible to attain uniformity of pickling action from bath to bath. Again, other non-oxidizing mineral acids than sulfuric acid may be employed in the pickle bath. Thus hydrochloric acid as well as other inorganic acids may be employed in the pickle bath in conjunction with the preferred class of inhibitors in the manner hereinbefore set forth.

What is claimed is:

1. A process of pickling a metal which comprises subjecting the metal to be pickled to the action of a mineral acid solution containing a small proportion of a thiourethane.

2. A process of pickling a metal which comprises subjecting the metal to be pickled to the action of a mineral acid solution containing a small proportion of a compound possessing the structure



40

wherein  $\text{R}_1$  and  $\text{R}_2$  are selected from the group consisting of hydrogen, alkyl, aralkyl and carbocyclic groups and  $\text{R}_3$  is an ester forming radical.

3. A process of pickling a metal which comprises subjecting the metal to be pickled to the action of a non-oxidizing mineral acid solution containing a small proportion of an N-carbocyclic thiourethane.

4. A process of pickling a metal which comprises subjecting the metal to be pickled to action of a non-oxidizing mineral acid solution containing a small proportion of an N-aryl thiourethane.

5. A process of pickling a metal which comprises subjecting the metal to be pickled to the action of a non-oxidizing mineral acid solution containing a small proportion of an N-phenyl thiourethane.

6. A process of pickling iron and steel products which comprises subjecting the metal to be pickled to the action of a sulfuric acid solution containing a small proportion of N-cyclohexyl thiourethane.

7. A process of pickling iron and steel products which comprises subjecting the metal to be pickled to the action of a sulfuric acid solution containing a small proportion of N-phenyl benzyl thiourethane.

8. A process of pickling iron and steel products which comprises subjecting the metal to be pickled to the action of a sulfuric acid solution containing a small proportion of N-phenyl butyl thiourethane.

45

50

55

60

65

70

75

2,201,488

3

9. A pickling bath for metal products which comprises a mineral acid solution containing a small proportion of a thiourethane.

10. A pickling bath for metal products which comprises a mineral acid solution containing a small proportion of a compound possessing the structure



wherein  $R_1$  and  $R_2$  are selected from the group consisting of hydrogen, alkyl, aralkyl and carbocyclic groups and  $R_3$  is an ester forming group.

11. A pickling bath for metal products which comprises a non-oxidizing mineral acid solution containing a small proportion of an N-carbo-cyclic thiourethane.

12. A pickling bath for metal products which

comprises a non-oxidizing mineral acid solution containing a small proportion of an N-aryl thiourethane.

13. A pickling bath for metal products which comprises a non-oxidizing mineral acid solution containing a small proportion of an N-phenyl thiourethane.

14. A pickling bath for metal products which comprises a sulfuric acid solution containing a small proportion of N-cyclohexyl thiourethane.

15. A pickling bath for metal products which comprises a sulfuric acid solution containing a small proportion of N-phenyl benzyl thiourethane.

16. A pickling bath for metal products which comprises a sulfuric acid solution containing a small proportion of N-phenyl butyl thiourethane.

MARION W. HARMAN.